

# UNITED STATES PATENT OFFICE.

JOSEPH L. R. HAYDEN, OF SCHENECTADY, NEW YORK, ASSIGNOR TO GENERAL ELECTRIC COMPANY, A CORPORATION OF NEW YORK.

## ARC-ELECTRODE AND PROCESS FOR MAKING IT.

1,093,182.

Specification of Letters Patent. Patented Apr. 14, 1914.

No Drawing.

Application filed August 17, 1908. Serial No. 443,797.

To all whom it may concern:

Be it known that I, JOSEPH L. R. HAYDEN, a citizen of the United States, residing at Schenectady, county of Schenectady, State of New York, have invented certain new and useful Improvements in Arc-Electrodes and the Process of Making Them, of which the following is a specification.

My invention relates to arc light electrodes and the process of compounding the same mainly of two or more metallic oxids in which the ingredients are uniformly mixed. Electrodes of this character are preferably but not exclusively used as cathodes in conjunction with anodes of carbon, or of copper, or other metal. The different metallic oxids, of which such electrodes are composed have ordinarily different degrees of fusibility, and owing to the incomplete mixture of the oxids obtained by the ordinary manner of making these electrodes, the different oxids fuse separately, that is to say, in succession, one after the other, in the pool which forms at the working end of the cathode, so that those compounds which fuse more readily are already in a fluid state when the more refractory ones are still solid. It follows from this that the more refractory compounds do not furnish to the arc the amount of vapor or gas which is due to the proportion of these compounds in the composition of the electrode. Thus, for instance, in an electrode compounded of magnetite, rutile, chromite, or the oxid of chromium, and possibly some other slight admixture, like fluorid of potassium, it happens that when the magnetite is in a perfectly fluid state at the working end of the cathode, the rutile is only imperfectly molten and the chromite may still be in a solid state. As a result of this the evolution of vapor from the rutile is retarded, by reason of the fact that it is behind the magnetite in fusibility. In this manner the arc is deprived of the luminosity which should be imparted to it by the titanium vapors. The effect of the dissimultaneous fusion of the component parts of the compound is not observable at the beginning of the operation, but after the cathode has been used for some time it manifests itself in the change of color and dimming of the arc. It may well be that the arc is maintained from the magnetite and rutile until these materials have been consumed at the point where the

arc is issued from the working end of the electrode, and the arc must then feed upon the chromite particles until these are consumed. During this stage the arc assumes the dull bluish tinge of the chromium arc. Its luminosity is diminished to some extent, and the arc becomes hotter. The higher temperature is deleterious to the positive electrode. I have found that this periodic change of color and dimming of the luminous arc, due to the different degrees of fusibility of its constituents, is mainly due to the incompleteness of the mixture obtained by the ordinary method of compounding such electrodes; and I found that if the ingredients employed in the composition of the electrodes are very intimately mixed, the different constituents of the same, although naturally of different degrees of fusibility, will practically fuse together as a unit, so that every constituent will give its proportional amount of vapors to the arc; and I have found that the requisite intimate mixture of these ingredients can be obtained in the following manner:—Instead of mixing the constituents of the electrode by grinding each separately and then mixing them mechanically, or by grinding them all together, which is the ordinary way of making an electrode of the character above described, and by which process the mixture is necessarily incomplete, I melt the ingredients together in a crucible, so that a practically homogeneous body is obtained which, upon cooling, becomes very brittle, and is then easily powdered to any degree of fineness. The mixture of the ingredients thus obtained is exceedingly uniform, and when filled in iron tubes or otherwise formed into pencils, and when these pencils are used as cathodes in electric arc lamps, the pool formed at the working end is composed of a fluid mixture of all the constituents of the electrode, since now all of them fuse at substantially the same time, and the evolution of vapors or gases from the same proceeds uninterruptedly, each constituent giving vapors in proportion to its proportional quantity present in the mixture. No periodic dimming and changing of color of light is observable in an electrode made in this manner.

In the ordinary electrode composed of magnetite, titanium oxid, chromite or chromium oxid, and possibly some potassium flu-

orid, the percentage of titanium oxid must be kept rather low, as the titanium dioxid has a low conductivity at ordinary temperatures, and when introduced by mechanically mixing is apt to form with the chromite a layer of slag, which becomes non-conducting when the arc is extinguished and the electrode allowed to cool. This interferes with the subsequent starting of an arc. With my process of compounding these ingredients, I am enabled to use a much higher percentage of titanium oxid than was heretofore used, as the intimate mixture of the ingredients results in a mass which is conducting even with a high percentage of titanium dioxid, and as the ingredients are consumed more uniformly, the layer of slag is not present. The added amount of titanium dioxid in the electrode is an advantage, since the titanium vapors impart to the arc a high degree of luminosity. I have found that with the above named ingredients, but with about ten per cent. more of titanium dioxid or rutile than has hitherto been practicable, a fluid mixture of the ingredients is obtained at about the melting point of cast iron. The substances fuse together to a black stony mass, which can be very easily powdered, since it is very brittle. It is then filled into the iron tube in the usual man-

ner, and thereby an electrode is obtained which gives increased steadiness of light and an increased efficiency.

What I claim as new and desire to secure by Letters Patent of the United States, is,—

1. An arc light electrode, the arc supporting body of which consists of the powder of a solidified fusion containing metallic compounds.

2. An arc light electrode, the arc supporting body of which consists of the powder of a solidified fusion containing metallic oxids.

3. An arc light electrode, the arc supporting body of which consists of the powder of a solidified fusion of magnetite, rutile, chromite and fluorid of potassium.

4. An arc light electrode consisting of an iron tube packed with the powder of a solidified fused mass containing metallic oxids.

5. An arc lamp electrode consisting of an iron tube packed with the powder of a solidified fused mass containing metallic oxids and a fluorid.

In witness whereof, I have hereunto set my hand this 8th day of August, 1908.

JOSEPH L. R. HAYDEN.

Witnesses:

BENJAMIN B. HULL,  
HELEN ORFORD.